

## United States Patent Office

2,941,949

Patented June 21, 1960

1

2,941,949

ACID BATHS FOR CLEANING AND  
PICKLING METALAlbert J. Saukaitis, Wayne, Pa., assignor to Amchem  
Products, Inc., Ambler, Pa., a corporation of Delaware

No Drawing. Filed May 14, 1957, Ser. No. 658,961

7 Claims. (Cl. 252—151)

XR -

This invention relates to the art of cleaning and pickling metal surfaces and is particularly concerned with the provision of a new method and bath for cleaning and pickling surfaces of mild steel, zinc (particularly galvanized steel) and aluminum.

As is well known to those skilled in the art, the cleaning and pickling of the metals mentioned is commonly effected by means of acid baths which remove scale or oxide from the surface and the principal object of my invention is to provide improved baths for this purpose.

The cleaning and pickling acids with which my invention is especially useful are those non-oxidizing mineral acids from the class which consists of sulphuric, phosphoric, hydrochloric, sulfamic, hydrofluoric and fluosilicic acids.

My invention resides in the discovery that the addition of a small amount of triphenyl sulfonium chloride to an acid cleaning or pickling solution of the class just described substantially prevents or retards the attack of the acid on the basis metal without interfering with the removal of scale or oxide from the surface.

In carrying out my invention the baths are normally used at conventional concentrations of acid and at customary temperatures. These factors, therefore, are familiar to the art and can be varied as desired within the practices which are customary in this field.

The quantity of triphenyl sulfonium chloride which I incorporate in such baths can vary but should, of course, be sufficient to substantially reduce the rate of acid attack on the basis metal while still accomplishing the desired cleaning and pickling. In general, only a relatively small amount of triphenyl sulfonium chloride is required and my experience indicates that this need be no greater than approximately 1% by weight of the bath, although this limit may be exceeded to a reasonable extent without, apparently, in any way impairing the desired results. As a practical matter, a useful amount for any particular acid or type of work can easily be determined by simple test within the knowledge of those skilled in this art.

By way of specific examples the following may be noted but they are in no sense to be considered as limiting. Certain commercial pickling procedures involve use of a 10% 66° Bé. sulfuric acid bath heated to approximately 180° F. A basic bath of this kind was prepared and to a portion of it was added 1/4% triphenyl sulfonium chloride. A succession of mild steel panels were then pickled in the bath for 1/2 hour each. Panels treated after the 1st, 3rd, 5th, 22nd, 24th, 26th and 28th hours of bath life were weighed before and after pickling and the weight loss recorded. These weight losses were respectively: 0.615, 0.665, 0.72, 0.75, 0.81, 0.748, and 0.764 gram per square foot per 1/2 hour immersion. The basic bath containing no inhibitor when used on identical steel panels caused a 72.5 gram per square foot weight loss per 1/2 hour immersion. The data, therefore, clearly illustrates

2

the value of my invention in inhibiting attack of the bath upon the metal and further demonstrates that iron buildup in the bath does not materially impair the efficiency of the inhibitor.

- 5 In another example a 3% sulfamic acid solution employing 1/2% by weight of triphenyl sulfonium chloride was used to pickle a galvanized steel panel. After remaining in the solution for 64 hours, the panel showed much less corrosion than an exactly similar panel pickled 10 in the same type of acid solution but containing a familiar commercial inhibitor especially recommended for use in the pickling of galvanized steel instead of the triphenyl sulfonium chloride of my invention. This was true even when the panel was left in the solution for as short a time as 2 hours instead of the 64 hours for the panel treated 15 with the bath of my invention.

In connection with sulfamic acid baths, I should like to point out that these are quite widely used in the cleaning of aluminum, particularly aluminum which is employed in the handling of milk. Such aluminum milk handling equipment frequently becomes completely encrusted with milk scale and it is customary to employ sulfamic acid to remove such scale but, unfortunately, this acid also seriously attacks the aluminum. However, 20 a cleaning solution consisting of 10 grams of sulfamic acid with sufficient water to make 100 cc. when inhibited with 1/10 gram triphenyl sulfonium chloride satisfactorily cleaned a severely encrusted aluminum vessel without substantial attack on the basis metal. This, therefore, 25 constitutes a preferred embodiment of my invention.

Still another example involved steel panels certain of which were immersed in a 75% phosphoric acid pickling solution containing 1% triphenyl sulfonium chloride. The bath was employed at 45° C., and the panels lost only 35 1.17 grams per square foot after 24 hours immersion, whereas, similar panels pickled in a similar but uninhibited phosphoric acid solution lost 209 grams per square foot after only 17.5 hours of immersion.

In conclusion, cleaning and pickling of metals according to my invention can be carried out with any of the procedures familiar in this art as by continuously passing the metal to be pickled (such as wire or sheets) through a number of baths in a regulated manner or by immersing the articles in the bath for a suitable period of time. The 40 temperature may be varied as indicated above, but ordinarily the baths of my invention are used at temperatures of from 140° to 190° F.

I claim:

1. A mineral acid bath for cleaning and pickling metal surfaces, said bath containing, as an inhibiting addition agent, an amount of triphenyl sulfonium chloride which is sufficient to reduce the rate of acid attack on metal.
2. The method of cleaning and pickling surfaces of steel, zinc and aluminum which consists in subjecting the surface to the action of a bath according to claim 1.
3. A bath of claim 1 wherein the quantity of triphenyl sulfonium chloride does not exceed 1% by weight of the bath.
4. The method of cleaning and pickling surfaces of steel, zinc and aluminum which consists in subjecting the surface to the action of a bath according to claim 3.
5. An acid bath for cleaning and pickling metal surfaces, said bath comprising acid from the class consisting of sulphuric, phosphoric, hydrochloric, sulfamic, hydrofluoric and fluosilicic acids and including triphenyl sulfonium chloride in an amount sufficient to reduce the rate of attack of the acid on the metal.
6. The acid bath of claim 5 in which the mineral acid is sulfamic acid.
7. The method of cleaning and pickling surfaces of

steel, zinc and aluminum which consists in subjecting the surface to the action of a bath according to claim 5.

References Cited in the file of this patent

UNITED STATES PATENTS

|           |                  |            |                |           |
|-----------|------------------|------------|----------------|-----------|
| 1,852,194 | Semon            | 252-151XR  | Apr. 5, 1932   | 2,220,451 |
| 1,877,504 | Grebe et al.     | 252-148XR  | Sept. 13, 1932 | 2,531,440 |
| 2,006,216 | MacArthur et al. | 252-148    | June 25, 1935  | 2,531,812 |
| 2,148,006 | Arveson          | 252-1424XR | Feb. 21, 1939  | 2,681,314 |
| 2,149,894 | Lieber et al.    | 222-153    | Mar. 7, 1939   | 2,698,781 |
| 2,178,353 | Werntz           | 266-67A    | Oct. 31, 1939  | 5         |

|                   |           |               |
|-------------------|-----------|---------------|
| Hunt              | 252-142   | Nov. 5, 1940  |
| Jordon            | 252-477   | Nov. 28, 1950 |
| Hauser            | 252-159   | Nov. 28, 1950 |
| Skinner           | 252-28    | June 15, 1954 |
| Meyer             | 252-142   | Jan. 4, 1955  |
| Funderburk et al. | 252-52    | Feb. 15, 1955 |
| Cardwell et al.   | 252-142XR | July 12, 1955 |
| Chiddix et al.    | 252-4528  | Aug. 21, 1956 |
| Pitt              | 266-67A   | July 30, 1957 |
| Beiswanger et al. | 252-448   | Nov. 26, 1957 |